

E. L. BURRELL,

METHOD OF TREATING THE FABRIC FOR POWER TRANSMISSION BELTS.

APPLICATION FILED FEB. 13, 1915.

1,218,052.

Patented Mar. 6, 1917.



Witnesses

M. H. Klant.

Walter F. Stone.

Inventor

Ernest L. Burrell,  
Bummler & Bummler  
Attns.

# UNITED STATES PATENT OFFICE.

ERNEST L. BURRELL, OF CHICAGO, ILLINOIS.

## METHOD OF TREATING THE FABRIC FOR POWER-TRANSMISSION BELTS.

1,218,052.

Specification of Letters Patent.

Patented Mar. 6, 1917.

Application filed February 13, 1915. Serial No. 7,946.

*To all whom it may concern:*

Be it known that I, ERNEST L. BURRELL, a citizen of the United States of America, and a resident of Chicago, county of Cook, and 5 State of Illinois, have invented certain new and useful Improvements in Methods of Treating the Fabric for Power-Transmission Belts, of which the following is a specification.

10 Cotton fabric specially woven and treated with various compositions, with a view to strengthening and preserving the fibers thereof, has long been used for power transmission purposes. The nature of the compositions used and the method of treating the fabric therewith have been varied and numerous. However, none of the belts so far produced has been suitable for use in many of the places where leather belts have heretofore been considered necessary, for the reason that the compositions used have either not materially increased the strength of the fibers, so as to render the material any more suitable for use, or have not preserved the 20 material against deterioration, or have actually caused a deterioration thereof.

The main object of this invention, therefore, is to provide an improved method of preparing cotton woven belting material for 30 use as power transmission belts, by treating the material with a new combination of ingredients which serve to strengthen and preserve the fibers of said material, and render the same impervious to and unaffected by 35 moisture.

In the accompanying drawing the figure represents a fragment of woven cotton belting material of the kind most suitable for use in making power transmission belting, 40 and with which the process hereinafter described is followed out. This is preferably a solid close-woven fabric woven with the desired number of layers to provide the necessary thickness. Thus, there are no stitches to come apart and weaken the belt. However, laminated material could be used with equal effectiveness so far as the action of the ingredients used in following out the process is concerned.

Although perfectly ripe cotton fiber consists of almost pure cellulose, the cells are filled with a somewhat gelatinous matter which in the untreated fabric is subject to oxidization and decay, and in time tends to deteriorate the fiber. In the compounds and

methods heretofore used in the treatment of woven cotton belting material, the attempt has been made to impregnate the fabric so as to isolate this foreign gelatinous matter from the action of air and moisture. 60

In my improved method of treating cotton woven belting material, the first step has been to neutralize this gelatinous matter by subjecting the material to the action of tannic acid in substantially the same manner 65 as that pursued in the tanning of hides. When thus infused with tannic acid the gelatinous matter is converted into a tough imputrescible substance, so that if it is thereafter exposed to air and moisture, it is unaffected. In addition, a considerable quantity of tannin is absorbed by the fibers and are thereby preserved against deterioration. It has also been found that this treatment increases the tensile strength of the material 75 about one-third.

An auxiliary step in the tanning process is to set the tannin with a mordant, such as tar-tar emetic (antimony oxy tartrate). This is done by preparing a fixing bath of about 80 two hundred pounds of water to which has been added about one-half per cent. of tar-tar-emetic. About one hundred pounds of the fabric is then immersed in the bath long enough for the desired action to take place. 85 This prevents the tannin from being freed from the fabric, as is otherwise likely to occur.

The next step is to impregnate the tanned fabric with a water-proofing compound 90 which is caused to penetrate the entire fibrous structure. The ingredients that can be used for this purpose are many and varied. However, there are certain characteristics which I have found this compound 95 should possess in order to produce belting having the desired qualities. In the first place, the compound should contain ingredients which are capable of giving weight or body to the fabric and which are unaffected by atmospheric changes, so that the treated material will not become either stiff or too pliable when exposed to cold or heat. On the other hand, the use of ingredients should be avoided, which of themselves are 105 subject to deterioration and which, by reason thereof, are likely to affect the fabric. The compound that I have found to possess these qualities is one made up of wax tailings, paraffin, and lubricating oil, com- 110

combined in substantially the following proportions:

|                 |          |
|-----------------|----------|
| Wax-tailings    | 900 lbs. |
| Paraffin        | 260 "    |
| Lubricating oil | 200 "    |

These products are mixed in a tank and heated to a temperature of from 200° to 225° F. The fabric is run through the solution in the tank, and readily becomes thoroughly impregnated therewith, whereupon it is rendered thoroughly water-proof and impervious to moisture.

These ingredients being mineral products are free from foreign putrescible substances, which is not the case with vegetable and animal oils. Therefore, belting material treated with this compound is not subject to deterioration by the action of any of the ingredients, but in fact, its preservation is increased. The lubricating oil is preferably a high grade cylinder oil, and is used primarily because it is not affected by the more usual low temperatures, and there is little danger of the belt losing its pliability in cold weather.

The fabric after being impregnated with this water-proofing compound presents an oily surface which will not afford the best frictional contact with the pulleys. The final step in this improved method, therefore, is to face the belt with a suitable dressing compound in order to increase its friction on the pulley faces and lengthen its wearing qualities. The dressing must be of such a character that it will penetrate the oily surface of the fabric treated in above manner so as to permanently adhere thereto. The following compound has been found to produce very satisfactory results in this respect:

|                     |          |
|---------------------|----------|
| Water               | 200 lbs. |
| Dry shellac         | 24 "     |
| Dry borax           | 6 "      |
| Dry asbestos powder | 10 "     |
| Dry pigment (green) | 100 "    |

The dressing is prepared by adding the borax and shellac to water and boiling. After the shellac has been dissolved the asbestos powder and pigment are added and thoroughly stirred into the liquid. The asbestos powder serves the double function of retarding the gravitation of the pigment in the solution and creating friction when a belt is put in service. This may be one of the many fire-proof substances such as asbestos, silica, fluorspar, etc. Silica, however, has been found to give the most satisfactory results.

The kind of pigment used is not vital so far as the action of the dressing is concerned, the color specified being used primarily for the purpose of making a distinctive appearance.

The water, shellac, and borax constitute an adhesive for applying and retaining the asbestos powder and pigment upon the surface of the belt.

The dressing is applied by brushing it on the surface of the belt or by running the belt through a tank containing the solution, the solution being thoroughly stirred to keep the pigment from gravitating. The dressing penetrates a slight distance into the fabric and will dry quickly leaving a part of elastic filament over the surface of the belt which will not crack or peel off, and is not affected by atmospheric changes. This coating or filament is impervious to water, oil, moisture, or any other substances that the belt may come in contact with, and prevents the same from reaching the fabric. However, the water-proofing compound tends to ooze out of the belt very slightly when the belt is running, but sufficiently to obtain a smooth wearing surface on the side of the belt next to the pulleys, so as to keep it in the best of condition.

It will be understood that the specific ingredients and other details of the process and product herein described, and the combination thereof may be modified by substitutions, omissions and additions without departing from the spirit of this invention as defined by the following claims.

I claim:

1. In the manufacture of power transmission belts from woven fiber belting material, the improved method of preparing the material which consists in subjecting it to the action of tannic acid, setting the tannin by means of a mordant, and then impregnating the same with a water-proofing compound.

2. In the manufacture of power transmission belts from woven fiber belting material, the improved method of preparing the material which consists in subjecting it to the action of tannic acid, setting the tannin by means of tartar emetic, and then impregnating the same with a water-proofing compound.

3. In the manufacture of power transmission belts from woven fiber belting material, the improved method of preparing the material which consists in subjecting it to the action of tannic acid and then impregnating the same with a heated water-proofing compound comprising substantially 66% wax tailings, 19% paraffin, and 15% lubricating oil.

4. In the manufacture of power transmission belts from woven fiber belting material, the improved method of preparing the material which consists in subjecting it to the action of tannic acid, impregnating the same with a water-proofing compound and then facing it with an asbestos dressing.

5. In the manufacture of power transmission belts from woven fiber belting material,

the improved method of preparing the material which consists in subjecting it to the action of tannic acid, impregnating the same with a water-proofing compound and then 5 facing it with an asbestos dressing compound containing a pigment.

6. In the manufacture of power transmission belts from woven fiber belting material, the improved method of preparing the mate-

10 rial which consists in subjecting it to the action of tannic acid, impregnating the same with a water-proofing compound and facing it with a shellac composition containing asbestos.

15 7. In the manufacture of power transmission belts from woven fiber belting material, the improved method of preparing the material which consists in subjecting it to the action of tannic acid, impregnating the same 20 with a water-proofing compound and facing it with a shellac composition containing asbestos and pigment.

8. In the manufacture of power transmission belts from woven fiber belting material, 25 the improved method of preparing the mate-

rial which consists in subjecting it to the action of tannic acid, impregnating the same with a water-proofing compound and facing it with a shellac composition containing substantially 10% shellac, 3% borax, and 87% 30 water with which has been combined, in substantially equal amounts by weight, a mixture of asbestos and pigment in the proportions of approximately 1 to 10.

9. In the manufacture of power transmission belts from woven fiber belting material, the improved method of preparing the material which consists in subjecting it to the action of tannic acid, impregnating it with a heated water-proofing compound comprising 35 paraffin and a high boiling mineral oil, and then facing the same with an asbestos dressing containing a pigment.

Signed at Chicago this 5th day of February, 1915.

ERNEST L. BURRELL.

Witnesses:

EDWIN PHELPS,  
C. M. FEIGEL.